

## UNITED STATES PATENT OFFICE

OTTO RÖHM, OF DARMSTADT, GERMANY

## TREATMENT OF HIDES

No Drawing. Application filed February 5, 1925, Serial No. 7,145, and in Germany April 1, 1924.

My invention refers to the treatment of hides, skins, pelts and furs, and more especially to the preparation of hides for the tanning.

As is well known to those skilled in the art, the raw or salted hides, in order to remove the hairs or bristles, are treated with a suitable depilatory, such as lime, which being slightly soluble in water does not give satisfactory results and requires many days' treatment. It has therefore been proposed to un-hair the hides by means of sulphides such as sodium sulphide which, however, while allowing of removing the hairs or bristles in a comparatively short time, at the same time acts on them in such a manner as to render them unfit for further use.

It is an object of my invention to provide means whereby the hides are acted upon in such manner that the hairs or bristles can easily be removed after a short treatment without however being injured and rendered unfit for further use.

To this end I subject the hides to a sequence of operations comprising a treatment with ammonia. I am aware that it has been proposed to employ ammonia for instance by exposing the hides to the combined action of ammonia and steam, but such treatment has proved to be ineffective, inasmuch as a uniform depilation cannot be obtained.

According to the present invention the hides, either raw or salted, are first treated with a salt of an alkali forming metal in the presence of an acid and thereafter with ammonia. The term salt of an alkali forming metal, wherever it occurs, is intended to include salts of the alkali metals, of the alkaline earths and of ammonia.

I prefer neutralizing the acid and rinsing with water before treating with ammonia. I prefer using hydrochloric acid or lactic acid, but other acids can be used with similar results and I may add the acid to the salt or salt solution at the beginning or at a later stage.

The operation of rinsing can however also be dispensed with, depilation being effected also without removing the salts. This is contrary to the practice generally followed of

freeing the hides from the salt contained therein, before proceeding with depilation, it being assumed that the presence of salts renders depilation more difficult. I have found that this is not the case and I therefore often dispense with washing or rinsing whereby much time is saved.

Preferably, tryptically active substances, for instance the pancreas enzymes, are caused to act on the hides either before or after treating with ammonia, in order to effect the bathing, to wash out the dirt and to further depilation without any extra bathing procedure. Preferably, an enzyme preparation is employed which is obtained by compressing the respective tissue (such as for instance the pancreas gland) with a view to recovering therefrom the liquor containing the enzymes (such as pancreas enzyme), this liquor being preferably mixed for absorption with a finely subdivided material such as wood meal. The preparations thus obtained form dry and stable products. I may, however, also employ the chopped or otherwise comminuted glands as such.

The treatment with ammonia may be carried out by fulling the hides in a watery solution of ammonia, part of which can however be replaced by other alkaline substances such as soda or potash. I have sometimes found it useful to employ ammonia in the form of a gas and preferably in statu nascendi by liberating it from a suitable salt capable of developing an easily decomposable ammonia compound or gaseous ammonia.

I may for instance employ a mixture of a salt of an alkali forming metal such as sodium chloride and an easily decomposable ammonia compound, such as ammonium chloride for the preparatory treatment of the hides, a suitable acid being added, and the ammonia required for depilation may then be liberated from the ammonia compound by adding a substance such as soda which will decompose the ammonium chloride, liberating ammonia.

After the hair has been removed, a plumping agent (for instance soda) can be added, and the plumping operation can be followed

by a bathing operating, a suitable bathing agent, for instance pancreas enzymes being added.

Instead of treating the hides with solutions of the salts or other substances, I can 5 also use these substances in solid state, the hide being first treated for instance with a mixture of a salt of an alkali forming metal such as sodium chloride, an ammonia salt such as ammonium chloride and an acid, for 10 instance lactic acid, and thereafter with a mixture of pancreas enzymes and soda, this latter being designed to liberate ammonia from the ammonium chloride.

In carrying out my invention I may for 15 instance proceed as follows:—

*Example 1*

100 kilos salted calfskins are fulled in 200 liters water, 20 kilos sodium chloride and 1 20 kilo lactic acid. The acid is then neutralized and 1 kilo of a preparation as aforesaid containing pancreas enzymes is added. After the lapse of a few hours, the hides are withdrawn from the bath and the salts are 25 removed by rinsing with water, whereupon they are fulled one hour in 100 liters water to which 16 kilos of a 25% solution of ammonia have been added. This treatment results in 30 a perfect depilation, the hairs being rendered easily removable.

*Example 2*

100 kilos salted calfskins are fulled with 200 liters water, 20 kilos sodium chloride 35 and 1 kilo lactic acid and are then allowed to remain in the solution for 24 hours. The acid is now neutralized, the salt solution is removed by rinsing and the hides are then fulled with 100 liters water to which are 40 added 4 kilos ammonia. The hairs can be removed after the lapse of an hour and the hides are then washed with water and treated with 1 kilo of a preparation containing pancreas enzymes.

45

*Example 3*

100 kilos salted calfskins are fulled with 300 liters water and 15 kilos sodium chloride. After the lapse of a day 1 kilo of a 30% 50 hydrochloric acid is added. After a further 24 hours the hides are removed from the solution and are fulled with 300 liters water to which have been added 12 kilos of an aqueous solution containing 25% by weight 55 of ammonia and 3 kilos soda. After the lapse of an hour the hairs can be removed.

*Example 4*

100 kilos salted calfskins are fulled a few 60 hours with 300 liters water, 15 kilos sodium chloride and 1 kilo of a preparation containing pancreas enzymes. 1 kilo of a 30% hydrochloric acid is then added. After 24 65 hours the acid is neutralized, the hides are removed from the solution and are now fulled

with a solution of 12 kilos of a watery solution containing 25% by weight of ammonia and 3 kilos potash in 300 liters water. The hides are ready for depilation after one hour's treatment.

*Example 5*

100 kilos salted calfskins are treated during 24 hours with 300 kilos water and 15 kilos sodium chloride, whereupon 1 kilo of a 30% hydrochloric acid is added. After a further 24 hours the hides are placed in a room filled with ammonia vapors. After remaining therein a few hours they are ready for depilation.

*Example 6*

100 kilos salted calfskins are fulled with 300 kilos water, 10 kilos sodium chloride and 10 kilos ammonium chloride. After 24 hours 1 kilo hydrochloric acid is added, after a further 24 hours the hides are removed from the solution and are fulled with a solution of 10 kilos soda in 300 liters water, the soda liberating ammonia in *statu nascendi* from the ammonium chloride still adhering to the 90 hides. After a few hours the hides are prepared for the removal of the hairs.

*Example 7*

100 kilos salted calfskins are first treated with a mixture of 10 kilos sodium chloride and 1 kilo lactic acid and thereafter with a mixture of 10 kilos soda, 10 kilos ammonium chloride and 1 kilo of the pancreas enzyme preparation hereinbefore described. The effect is substantially the same as described with reference to the wet treatment.

I wish it to be understood that I do not desire to be limited to the exact substances, proportions and sequence of operations specifically described, as obvious modifications will occur to a person skilled in the art.

I claim:—

1. The method of treating hides preparatory to tanning, comprising treating the hides first with a solution of a salt of an alkali forming metal and an acid and then with ammonia.

2. The method of treating hides preparatory to tanning, comprising treating the hides first with a salt of an alkali forming metal and an acid, neutralizing said acid and then treating with ammonia.

3. The method of treating hides preparatory to tanning, comprising treating the hides first with a salt of an alkali forming metal and an acid and then with ammonia, a tryptic active substance being caused to act on the hide.

4. The method of treating hides preparatory to tanning, comprising treating the hides first with a salt of an alkali forming metal and an acid and then with ammonia, pancreas enzyme being caused to act on the hide.

5. The method of treating hides preparatory to tanning, comprising treating the hides first with a salt of an alkali forming metal and an acid, neutralizing said acid and then 5 treating with ammonia, a tryptically active substance being caused to act on the hide.
6. The method of treating hides preparatory to tanning, comprising treating the hides first with a salt of an alkali forming 10 metal and an acid, neutralizing said acid and then treating with ammonia, and causing pancreas enzyme to act on the hide.
7. The method of treating hides preparatory to tanning, comprising treating the hides 15 first with a salt of an alkali forming metal and an acid, neutralizing said acid, rinsing and then treating with ammonia, and causing a tryptically active substance to act on the hide.
20. 8. The method of treating hides preparatory to tanning, comprising treating the hides first with a salt of an alkali forming metal and an acid and then with ammonia in statu nascendi.
25. 9. The method of treating hides preparatory to tanning, comprising treating the hides first with a salt of an alkali forming metal and an acid and then with ammonia gas.
30. 10. The method of treating hides preparatory to tanning, comprising treating the hides first with a salt of an alkali forming metal and an acid, neutralizing said acid, rinsing and then treating with ammonia and another alkaline compound, and causing pancreas 35 enzyme to act on the hide.

In testimony whereof I affix my signature.

OTTO RÖHM.

40

45

50

55

60

65